# EUROPEAN PATENT SPECIFICATION

(11) **EP 1 506 857 B1**
(45) Date of publication and mention of the grant of the patent: **25.04.2007**
(21) Application number: 04078163.5
(22) Date of filing: 08.06.1999
(51) Int. Cl.: B41C 1/10, B41M 5/36

(54) **Positive-working thermal imaging element and positive-working lithographic printing plate precursor**
Positiv arbeitendes thermisches bilderzeugendes Element und positiv arbeitender lithographischer Druckplattenvorläufer
Elément thermique travaillant en positif et formateur d'images et plaque d'impression lithographique travaillant en positif

(30) Priority: 23.06.1998 US 90300 P; 29.04.1999 US 301866
(43) Date of publication of application: 16.02.2005
(62) Divisional of application: 99928429.2
(73) Proprietor: EASTMAN KODAK COMPANY, Rochester, New York 14650-2201 (US)
(72) Inventor: Shimazu, Ken-Ichi, Briarcliff Manor New York 10704 (US); Patel, Jayanti, Carlstadt, New Jersey 07072 (US); Saraiya, Shashikant, Parlin New Jersey 08857 (US); Merchant, Nishith, North Bergon New Jersey 07047 (US); Savariar-Hauck, Celin, 37534 Badenhausen (DE); Timpe, Hans-Joachim, 37520 Osterode (DE); McCullough, Christopher, Fort Collins Colorado 80526 (US)
(74) Representative: Haile, Helen Cynthia

(56) References cited:
- EP-A1- 0 864 420
- EP-A1- 0 908 779
- EP-A1- 0 943 451
- EP-A2- 0 678 380

## Description

The present invention relates to positive-working thermal imaging elements and positive-working thermal lithographic printing plates which are imaged with an infrared laser and processed with an aqueous developer.

U.S. 5,493,971 discloses lithographic printing constructions which include a grained-metal substrate, a protective layer that can also serve as an adhesion-promoting primer, and an ablatable oleophilic surface layer. In operation, imagewise pulses from an imaging laser interact with the surface layer, causing ablation thereof and, probably, inflicting some damage to the underlying protective layer as well. The imaged plate may then be subjected to a solvent that eliminates the exposed protective layer, but which does no damage either to the surface layer or to the unexposed protective layer lying thereunder.

A heat-sensitive imaging element for making positive-working lithographic printing plates is disclosed in EP-A-0 864 420 (published 16 September 1998) and prior art according 54(3) and (4) EPC. The imaging element disclosed comprises a lithographic base, a layer comprising a polymeric material which is soluble in an aqueous alkaline solution and an IR-radiation sensitive second layer. Upon image-wise exposure and absorption of IR-radiation in the second (top) layer, the capacity of the aqueous alkaline solution to penetrate and/or solubilize the second layer is changed. Image-wise exposure can be performed with an infrared laser with a short as well as with a long pixel dwell time.

EP-A-0 678 380 describes a lithographic printing construction including a grained-metal substrate, a protective layer that can serve as an adhesion-promoting primer and an ablatable oleophilic surface layer, which may contain an IR-absorbing compound.

EP-A-0 908 779 (published 14 April 1999) and prior art according 54(3) and (4) EPC describes a thermal lithographic printing plate having a first alkaline-soluble layer and a top layer unpenetrable for an alkaline developer containing SiO₂ as silicate, and which may contain a compound capable of turning light to heat, preferably carbon black.

EP-A-0 943 451 (published 22 September 1999) and prior art according 54(3) and (4) EPC describes a thermal lithographic printing plate also comprising a first alkaline-soluble layer and a top layer unpenetrable for or insoluble in an alkaline developer containing SiO₂ in the form of silicates, characterised in that the first layer and the top layer comprise a compound capable of converting IR-light into heat.

Although advances have been made in the preparation of heat-sensitive elements for the production of lithographic printing plates, there remains a need for such elements having improved sensitivity to infrared laser imaging devices. There is also a need for longer shelf-life with wider development latitude and wider exposure latitude.

### SUMMARY OF THE INVENTION

These needs are met by the present invention which in a first aspect is a positive-working thermal imaging element comprising;
A. a substrate; and
B. a thermally sensitive composite layer structure having an inner surface contiguous to the substrate and an outer surface, the composite layer structure comprising:
   (a) a first layer having the inner surface, the first layer comprising a first polymeric material and a photoconversion material, wherein the first polymeric material is soluble or dispersible in an aqueous solution; and
   (b) a second layer having the outer surface, the second layer comprising a second polymeric material, wherein the second layer is insoluble in the aqueous solution, wherein the first layer, containing the photothermal conversion material, is applied first and the second layer, not containing a photothermal conversion material, is subsequently applied; and wherein, upon imagewise heating of the composite layer structure, the composite layer structure is provided with heated portions and complementary unheated portions, wherein the heated portions have an increased rate of removal in the aqueous solution.

In addition, the present invention may be defined in a second aspect as a positive-working, lithographic printing plate precursor which is the positive-working thermal imaging element of the first aspect of the invention, wherein the substrate is a hydrophilic substrate and the outer surface is outer oleophilic surface.

A third aspect of this invention is a method for forming a planographic printing plate comprising the steps, in the order given:
I) providing a lithographic printing plate precursor of the second aspect;
II) imagewise exposing the composite layer structure to thermal energy to provide exposed portions and complementary unexposed portions in the composite layer structure, wherein the exposed portions are selectively removable by the aqueous solution; and
III) applying the aqueous solution to the outer oleophilic surface to remove the exposed portions to produce an imaged lithographic printing plate having uncovered hydrophilic areas of the hydrophilic substrate and complementary ink receptive areas of the outer oleophilic surface. In an added embodiment of the method of this invention, the imaged lithographic printing plate is uniformly exposed to thermal energy after step III.

In a further embodiment of this invention the first layer of the thermal imaging element also contains a photohardenable material activatable by ultraviolet radiation. In use, the thermal imaging element of this embodiment is imaged and developed according to the method of this invention to form the imaged lithographic printing plate. The imaged lithographic printing plate may then be uniformly exposed to ultraviolet radiation.

In of each of the embodiments of this invention the aqueous solution preferably has a pH of about 6 or greater; the first polymeric material preferably is insoluble in an organic solvent, and the second polymeric material is preferably soluble in the organic solvent. The element is preferably imagewise exposed with a radiant source of energy such as an infrared emitting laser. The second layer applied is free of the photothermal conversion material.

### DETAILED DESCRIPTION OF THE INVENTION

This invention relates to an imaging element which can be imaged with thermal energy. More particularly, this invention relates to thermal lithographic printing plates, which can be imaged by thermal energy typically by imagewise exposure with an infrared emitting laser, a thermal printing head, or the like. The lithographic plates described in this invention are made up of a hydrophilic substrate, typically an aluminum or polyester support, and adhered thereto, a thermally sensitive composite layer structure typically composed of two layer coatings. An aqueous developable polymeric mixture typically containing a photothermal conversion material is coated on the hydrophilic substrate to form the first layer. The second layer is composed of one or more non-aqueous soluble polymeric materials which are soluble or dispersible in a solvent which does not dissolve the first layer. In the positive-working thermal imaging element of this invention, the term "photothermal conversion material" is intended to be one or more thermally sensitive components which absorb incident radiation and convert the radiation to thermal energy. Typically, the photothermal conversion material is an "infrared absorbing" compound.
The second layer does not contain a photothermal conversion material material. As used herein, the term "thermally sensitive" is intended to be synonymous with the term "heat sensitive", and the term "image area(s)" is intended to mean the surface area(s) of the imaged plate which is ink-receptive. The plate is exposed in non-image area(s), i.e., areas outside the "image areas" which are not ink-receptive, typically with an infrared laser or a thermal print head. Upon aqueous development of the imaged plate, the exposed portions are developed away thus exposing hydrophilic surfaces of the substrate which are receptive to conventional aqueous fountain solutions. The second layer composed of ink-receptive image areas, protects the underlying aqueous-soluble coating areas from the aqueous developer. In the following description, the invention will be illustrated using infrared radiation, and infrared absorbing material as the photothermal conversion material, but is not intended to be limited thereby.

In preferred embodiments the following features, described under the headings which follow, are present.

### Plate Construction

The plate construction of the present invention includes a composite layer structure supported by a substrate. The composite layer structure contains at least an ink-receptive, aqueous-insoluble second layer overlying an aqueous-soluble infrared absorbing layer which is adhered to the surface of the substrate. The composite structure may additionally contain intermediate layers such as substrate subbing layers to enhance hydrophilicity or adhesion to the composite structure, or an adhesion promoting interlayer between the second layer and the infrared absorbing layer.

### Substrate

Hydrophilic substrates which may be used in the planographic plate of this invention may be any sheet material conventionally used to prepare lithographic printing plates such as metal sheet materials or polymeric sheet material. A preferred metal substrate is an aluminium sheet. The surface of the aluminium sheet may be treated with metal finishing techniques known in the art including brushing roughening, electrochemical roughening, chemical roughening, anodizing, and silicate sealing and the like. If the surface is roughened, the average roughness Ra is preferably in the range from 0.1 to 0.8 µm, and more preferably in the range from 0.1 to 0.4 µm. The preferred thickness of the aluminium sheet is in the range from about 0.0127 cm (0.005 inch) to about 0.0508 cm (0.020 inch). The polymeric sheet material may be comprised of a continuous polymeric film material, a paper sheet, a composite material or the like. Typically, the polymeric sheet material contains a sub-coating on one or both surfaces to modify the surface characteristics to enhance the hydrophilicity of the surface, to improve adhesion to subsequent layers, to improve planarity of paper substrates, and the like. A preferred polymeric substrate comprises polyethylene terephthalate.

### Thermally-Sensitive Composite Layer Structure

First Layer: The first layer of the composite layer structure is composed of a polymeric material and a photothermal conversion material such as an infrared absorbing compound, in which the polymeric material is soluble or dispersible in an aqueous solution preferably having a pH of about 6 or greater, i.e., in a slightly acidic, neutral or alkaline aqueous solution. Optionally, the first layer may contain a photohardenable material in addition to the thermal conversion material. Useful polymeric materials contain acid functionality and may be composed of one or more polymers or resins. Such polymers and resins include carboxy functional acrylics, acrylics which contain phenol groups and/or sulfonamide groups, cellulosic based polymers and copolymers, vinyl acetate/crotonate/vinyl neodecanoate copolymers, styrene maleic anhydride copolymers, polyvinyl acetals, phenolic resins, maleated wood rosin, and combinations thereof. Typically two polymers are used in combination to achieve the desirable solubility in a wholly aqueous solution having a pH of about 6 or greater and typically between about 8 and about 13.5. A further criterion for the polymeric material, is that it is preferably insoluble in an organic solvent for the second layer hereinafter discussed.

In this invention, the first layer contains a photothermal conversion material such as an infrared absorber. An infrared absorber may be selected from either a dye or pigment. A primary factor in selecting the infrared absorber is its extinction coefficient which measures the efficiency of the dye or pigment in absorbing infrared radiation in accordance with Beer's Law. The extinction coefficient must have a sufficient value in the wavelength region of infrared radiation exposure usually from 780 nm to 1300 nm. Examples of infrared absorbing dyes useful in the present invention include, Cyasorb IR 99 and Cyasorb IR 165 (both available from Glendale Protective Technology), Epolite IV-62B and Epolite III-178 (both available from the Epoline Corporation), PINA-780 (available from the Allied Signal Corporation), Spectra IR 830A and Spectra IR 840A (both available from Spectra Colors Corporation), ADS 830A and ADS 1060A (ADS Corp) and EC 2117 (FEW Wolfen). Examples of infrared absorbing pigments are Projet 900, Projet 860 and Projet 830 (all available from the Zeneca Corporation). Carbon black pigments may also be used. Carbon black pigments are particularly advantageous due to their wide absorption bands since such carbon black-based plates can be used with multiple infrared imaging devices having a wide range of peak emission wavelengths.

In addition to the photothermal conversion material, the first layer may also contain a photohardenable material which is activatable by ultraviolet radiation. With the addition of the photohardenable material, printing plates with high press life and resistance to press room chemicals are produced. As used herein the term "photohardenable" material is intended to mean any component or group of components which, upon activation by ultraviolet radiation forms a matrix within the first layer by polymerization and/or crosslinking, so as harden and/or insolubilize the first layer; and/or to interact with surfaces of adjacent layers to increase adherence thereto. The photohardenable material may contain a photopolymerizable component, a photocrosslinkable component, or a combination thereof. Such photohardenable materials may additionally contain a photoinitiating system and/or a photosensitizing system. Without being bound by any particular theory, it is believed that the photohardenable material may form a matrix independent of the first polymeric material; may function to crosslink the first polymeric material; may function to chemically bond the first layer to the second layer; or a combination thereof. Typical photohardenable materials include diazonium polycondensation products, photoinitiated free radical polymerizable systems, hybrid combinations of diazonium polycondensation products and photoinitiated free radical polymerizable systems, cationically or anionically photopolymerizable systems, and systems which undergo photocrosslinking by photodimerization or photocycloaddition. Typically such photohardenable material contain a photoinitiating system, a photosensitizing system or a combination thereof. Such photoinitiating systems include conventional photoinitiators which form free radicals or ionic catalysts upon exposure to ultraviolet radiation. Such photosensitizing systems include conventional photosensitizing compounds which extend the effective spectral region of the photoinitiating system into the near ultraviolet and visible spectral region. Preferred among these photohardenable materials are those based on diazonium polycondensation products and systems which undergo photocycloaddition. Examples of such diazonium polycondensation products are described in U.S. Patent 4,687,727. A preferred product is derived from polycondensation of 3-methoxydiphenylamine-4-diazonium sulfate and 4,4'-bis-methoxymethyldiphenylether, isolated as the mysitylene sulfonate salt, and available from Panchim as Nega 107. Systems based on photocycloaddition are described in U.S. Patent 5,112,743, EP A 368 327 and DE 198 47 616.7. The effective spectral region of the latter systems can be extended into the near ultraviolet and visible regions using photosensitizers as described in DE 42 31 324 and DE 26 26 769. Preferred photosensitizers are thioxanthone derivatives.

Second Layer: The second layer of the composite layer structure, i.e. the top layer, contains as an essential ingredient a polymeric material which is preferably ink-receptive, is insoluble in the aqueous solution preferably having a pH of about 6 or greater, and is preferably soluble or dispersible in a solvent such as an organic solvent or an aqueous solvent dispersion. Useful polymers of this type include acrylic polymers and copolymers; polystyrene; styrene-acrylic copolymers; polyesters, polyamides; polyureas; polyurethanes; nitrocellulosics; epoxy resins; and combinations thereof. Preferred are polymethylmethacrylate and polystyrene. The second layer may also contain a dye or pigment, such as a printout dye added to distinguish the exposed areas from the unexposed areas during processing; or a contrast dye to distinguish image areas in the finished imaged plate. The second layer may also contain polymeric particles which are incompatible with the second polymeric material. As used herein the term "incompatible" is intended to mean that the polymeric particles are retained as a separate phase within the second polymeric material. Typically, the polymeric particles have an average diameter between about 0.5 µm and about 10 µm. Preferred polymeric particles of this type are poly tetrafluoroethylene particles. The presence of such polymeric particles improves scratch resistance of the composite layer and surprisingly enhances exposure latitude for processing the plate. Typically, the second layer is substantially free of ionic groups.

### Plate Precursor Preparation

The composite layer structure may be applied to the substrate by sequentially applying the first layer and then the second layer using conventional coating or lamination methods. It is important to avoid intermixing the two layers which tends to reduce the sensitivity. Regardless of the method of application, the first layer of the applied composite has an inner surface which is contiguous to the substrate, and the second layer of the applied composite has an outer surface.

The first layer containing a photoconversion material may be applied to the hydrophilic substrate by any conventional method. Typically the ingredients are dissolved or dispersed in a suitable coating solvent, and the resulting solvent mixture is coated by known methods such as by whirl coating, bar coating, gravure coating, roller coating, and the like. Suitable coating solvents include alkoxyalkanols such as 2-methoxyethanol; ketones such as methyl ethyl ketone; esters such as ethyl acetate or butyl acetate; and mixtures thereof.

The second or top layer not containing a photoconversion material may be applied to the surface of the thermal conversion first layer by any conventional method such as those described above. Typically the ingredients are dissolved or dispersed in a suitable organic coating solvent which is not a solvent for the thermal conversion layer. Suitable coating solvents for coating the second layer include aromatic solvents such as toluene and mixtures of aromatic solvents with alkanols such as a 90:10 weight ratio of toluene and butanol.

Alternatively, the first layer, the second layer or both layers may be applied by conventional extrusion coating methods from a melt mixture of layer components. Typically, such a melt mixture contains no volatile organic solvents.

### Plate Imaging and Processing

The thermal digital lithographic printing plate precursor is imaged by the method comprising the following steps. First a lithographic printing plate precursor is provided which comprises a hydrophilic substrate and adhered thereto, a composite layer structure having an inner surface contiguous to the hydrophilic substrate and an outer oleophilic, ink-receptive surface. The composite layer structure comprises a first layer which forms the inner surface of the composite layer structure and a second layer which forms the outer surface of the composite layer structure. The first layer comprises a first polymeric material and a photothermal conversion material, as previously described, in which the first polymeric material is preferably soluble or dispersible in an aqueous solution having a pH of about 6 or greater, and insoluble in an organic solvent. The second layer consists essentially of a second polymeric material, as previously described, which is soluble in the organic solvent, wherein the second layer is insoluble in the aqueous solution. Next the composite layer structure is imagewise exposed to thermal energy to provide exposed portions, or areas, and complementary unexposed portions, or areas, in the composite layer structure. The exposed portions surprisingly are selectively removable by the aqueous solution. Finally, the aqueous solution is then applied to the outer oleophilic surface to remove the exposed portions of the composite layer structure to produce an imaged lithographic printing plate. The resulting imaged lithographic printing plate has uncovered hydrophilic areas of the hydrophilic substrate and complimentary ink receptive areas of the outer oleophilic surface. While not being bound by any particular theory, selective removability of the exposed portions is believed to result from an increased rate of dissolution or dispersibility of the first layer in the aqueous solution, from enhanced permeability of the second layer to the aqueous solution or to a combination thereof.

The lithographic plate precursor of this invention and its methods of preparation have already been described above. This plate may be imaged with a laser or an array of lasers emitting infrared radiation in a wavelength region that closely matches the absorption spectrum of the first infrared absorbing layer. Suitable commercially available imaging devices include image setters such as a Creo Trendsetter (available from the CREO Corporation, British Columbia, Canada) and a Gerber Crescent 42T (available from the Gerber Corporation). While infrared lasers are preferred other high intensity lasers emitting in the visible or ultraviolet may also be used to image the lithographic plate of this invention. Alternatively, the lithographic plate precursor of this invention may be imaged using a conventional apparatus containing a thermal printing head or any other means for imagewise conductively heating the composite layer such as with a heated stylus, with a heated stamp, or with a soldering iron as illustrated in the following examples.

When portions of the composite layer structure are exposed to infrared radiation, they become selectively removable by an aqueous developer liquid and are removed thereby. The developer liquid may be any liquid or solution which can both penetrate the exposed areas and dissolve or disperse the exposed areas of the infrared absorbing layer without substantially affecting the complimentary unexposed portions of the composite layer structure. Useful developer liquids are the aqueous solutions having a pH of about 6 or above as previously described. Preferred developer solutions are those that have a pH between about 8 and about 13.5. Useful developers include commercially available developers such as PC3000, PC955, PC956, and PC9000 aqueous alkaline developers each available from Kodak Polychrome Graphics, LLC. Typically the developer liquid is applied to the imaged plate by rubbing or wiping the second layer with an applicator containing the developer liquid. Alternatively, the imaged plate may be brushed with the developer liquid or the developer liquid may be applied to the plate by spraying the second layer with sufficient force to remove the exposed areas. Alternatively, the imaged plate can be soaked in the developer liquid, followed by rubbing or brushing the plate with water. By such methods a developed printing plate is produced which has uncovered areas which are hydrophilic and complimentary areas of the composite layer, not exposed to infrared radiation, which are ink receptive.

Although lithographic printing plates having high press life with good ink receptivity are produced at high imaging speeds by the method of this invention, press life surprisingly is further enhanced by uniformly exposing the imaged lithographic printing plate to thermal energy after it has been developed in step III. Such a uniform thermal exposure may be carried out by any conventional heating technique, such as baking, contact with a heated platen, exposure to infrared radiation, and the like. In a preferred mode for post development thermal exposure, the developed imaged lithographic printing plate is passed through a baking oven at 240° C for 3 minutes after treatment with a baking gum.

When the first layer of the lithographic printing plate precursor element contains a photohardenable material, the developed, imaged lithographic printing plate may be uniformly exposed to ultraviolet radiation to further enhance press life and resistance to press room chemicals. Such post development flood exposures may be carried out using any conventional ultraviolet exposure source. In a typical post development flood exposure, the developed, imaged plate is placed in a conventional exposure device such as a 5W Theimer device for 20 seconds. As used herein, the term "ultraviolet radiation" is intended to include actinic radiation within the spectral region from about 250 nm to about 420 nm with the near ultraviolet spectral region from about 360 nm to about 400 nm being preferred.

The thermal lithographic printing plate of the present invention will now be illustrated by the following examples, but is not intended to be limited thereby.

### Example 1

A lithographic printing plate was prepared as follows:
First Layer: 2.5 g of 28-2930 copolymer (vinyl acetate/crotonates/ vinyl neodecanoate copolymer from National Starch and Chemical Co.) and 2.5 g of Scripset-550 (styrene maleic anhydride copolymer from Monsanto) were dissolved in 50 mL of 2-methoxyethanol and 50 mL methyl ethyl ketone solvent mix. 0.9 g. of ADS-830A dyes (American Dye Source Inc.) was added to this solution and stirred until all the ingredients were completely dissolved. The solution was then coated on an aluminum lithographic substrate to achieve a 2.0 g/m² coating.
Second layer: 13.2 g of A-21 (a 30% solution of polymethylmethacrylate (PMMA) in toluene/butanol 90:10 solvent mixture from Rohm & Haas) was dissolved in 190 g. of toluene. The solution was stirred and then coated on top of the above mentioned first layer coated plate.

The plate precursor was laser imaged on a Creo Trendsetter thermal exposure device having a laser diode array emitting at 830 nm with a dose of 100 to 300 mJ/cm². Upon alkali development with positive developer PC3000 (from Kodak Polychrome Graphics) having a pH of about 13.5, laser exposed areas of both the bottom and second layers were removed without affecting the unexposed areas of either layer.

When the plate precursor was prepared using Epolite III-178 dye (Epolin Inc.) in place of ADS-830A dye in the first layer, similar results were obtained following thermal imaging with a Gerber Crescent 42T exposure device, emitting at 1064 nm, and development as above.

When the plate precursor was thermally imaged with a Weller soldering iron (EC2100M), followed by development in an aqueous solution of sodium metasilicate pentahydrate (14 wt%), a positive image was similarly obtained. Similar results were obtained by scanning the coating or the substrate side of the plate precursor with the soldering iron at a rate of 10cm/s.

### Example 2

A lithographic printing plate was prepared as follows:
First Layer: 2.5 g. of SMA-1000 polymer (styrene maleic anhydride copolymer from ARCO Chemical) and 2.5 g. of PN-430 resin (phenolic resin from American Hoeschst) were dissolved in 50 mL of 2-methoxyethanol and 50 mL of methyl ethyl ketone solvent mix. 0.9 g. ADS-830A dye was added to this solution. The solution was stirred to dissolve all three components completely and was then coated on a lithographic substrate to achieve 2.0 g/m² coating weight using a whirl coater.
Second layer: 13.2 g. of A-21 was dissolved on 190 g. of toluene. The solution was stirred and then coated on top of the above mentioned first layer coated plate.

This plate was laser imaged on a Creo Trendsetter system as described in Example 1. Upon alkali development with positive developer PC3000, laser exposed areas of both the first and second layers were removed without affecting the unexposed areas of either layer.

In accordance with Example 1, similar results were obtained when ADS-830A dye was replaced by Epolite III-178 dye in the first layer and the plate precursor was exposed in the Gerber Crescent 42T device.

### Example 3

A lithographic printing plate was prepared as follows:
First Layer: 2.5 g of SD-140 resin, a phenol novolac resin, and 2.5 g. of 28-2930 copolymer were dissolved in 50 mL of 2-methoxyethanol and 50 mL of methyl ethyl ketone solvent mix. 0.9g. ADS-830 dye was added to this solution. The solution was stirred to dissolve all three components completely. The solution was then coated on lithographic substrate to achieve 2.0g/m² coating weight using a whirl coater.
Second layer: A 2% solution of Acryloid B-44 resin, an acrylic copolymer from Rohm & Haas having a Tg =60°C, in toluene was applied on top of the above mentioned first layer coated plate.

This plate was laser imaged on a Creo Trendsetter system as described in Example 1. Upon alkali development with positive developer PC3000, laser exposed areas of both the first and second layers were removed without affecting the unexposed areas of either layer.

In accordance with Example 1, similar results were obtained when ADS-830A dye was replaced by Epolite III-178 dye in the first layer and the plate precursor was exposed in the Gerber Crescent 42T device.

### Example 4

A lithographic printing plate was prepared as follows:
First Layer: 2.5 g. of cellulose acetate phthalate and 2.5 g. of 28-2930 copolymer were dissolved in 50 mL of 2-methoxyethanol and 50 mL of methyl ethyl ketone solvent mix. 0.9 g. ADS-830 dye was added to this solution. The solution was stirred to dissolve all three components completely. A solution was then coated on lithographic substrate to achieve 2.0 g/m² coating weight using a whirl coater.
Second layer: A 2% solution of Acryloid B-66 resin (an acrylic copolymer from Rohm & Haas having a Tg = 50° C) in toluene was applied on top of the above mentioned first layer coated plate.

This plate was laser imaged on a Creo Trendsetter system as described in Example 1. Upon alkali development with positive developer PC3000, laser exposed areas of both the first and second layers were removed without affecting the unexposed areas of either layer.

In accordance with Example 1, similar results were obtained when ADS-830A dye was replaced by Epolite III-178 dye in the first layer and the plate precursor was exposed in the Gerber Crescent 42T device.

### Example 5

A lithographic printing plate was prepared as follows:
First Layer: 2.5 g. of Carboset-500 (an acrylic copolymer from Goodrich) and 2.5 g. of 28-2930 copolymer were dissolved in 50 mL of 2-methoxyethanol and 50 mL of methyl ethyl ketone solvent mix. 0.9 g. ADS-830 dye was added to this solution. The solution was stirred to dissolve all three components completely. The solution was then coated on a lithographic substrate to achieve 2.0 g/m² coating weight using a whirl coater.
Second layer: A 2% solution of Acryloid B-82 (an acrylic copolymer from Rohm & Haas having a Tg = 35° C) in toluene was applied on top of the above mentioned first layer coated plate.

This plate was laser imaged on a Creo Trendsetter system as described in Example 1. Upon alkali development with positive developer PC3000, laser exposed areas of both the first and second layers were removed without affecting the unexposed areas of either layer.

In accordance with Example 1, similar results were obtained when ADS-830A dye was replaced by Epolite III-178 dye in the first layer and the plate precursor was exposed in the Gerber Crescent 42T device.

### Example 6

A lithographic printing plate was prepared as follows:
First Layer: 2.5 g. of Scripset-540 (styrene maleic anhydride copolymer from Monsanto) and 2.5 g. of 28-2930 copolymer were dissolved in 50 mL of 2-methoxyethanol and 50 mL of methyl ethyl ketone solvent mix. 0.9 g. ADS-830A dye was added to this solution. The solution was stirred to dissolve all three components completely. The solution was then coated on a lithographic substrate to achieve 2.0 g/m² coating weight using a whirl coater.
Second layer: A 2% solution of Acryloid B-84 resin (an acrylic copolymer from Rohm & Haas having a Tg = 50° C) in toluene was applied on top of the above mentioned first layer coated plate.

This plate was laser imaged on a Creo Trendsetter system as described in Example 1. Upon alkali development with positive developer PC3000, laser exposed areas of both the first and second layers were removed without affecting the unexposed areas of either layer.

In accordance with Example 1, similar results were obtained when ADS-830A dye was replaced by Epolite III-178 dye in the first layer and the plate precursor was exposed in the Gerber Crescent 42T device.

### Example 7

A lithographic printing plate was prepared as follows:
First Layer: 2.5 g. of Scriptset-550 and 2.5 g. of 28-2930 copolymer were dissolved in 50 mL of 2-methoxyethanol and 50 mL of methyl ethyl ketone solvent mix. 0.9 g. ADS-830 dye was added to this solution. The solution was stirred to dissolve all three components completely. The solution was then coated on a lithographic substrate to achieve 2.0 g/m² coating weight using a whirl coater.
Second layer: A 2% solution of polystyrene in toluene was applied on top of the above mentioned first layer coated plate.

This plate was laser imaged on a Creo Trendsetter system as described in Example 1. Upon alkali development with positive developer PC3000, laser exposed areas of both the first and second layers were removed without affecting the unexposed areas of either layer.

In accordance with Example 1, similar results were obtained when ADS-830A dye was replaced by Epolite III-178 dye in the first layer and the plate precursor was exposed in the Gerber Crescent 42T device.

### Example 8

A lithographic printing plate was prepared as follows:
First Layer: A carbon dispersion was made by dispersing 15 g carbon black (Spezialschwarz 250 from Degussa) in a solution of 30 g of PD 140 A resin (cresol novolac resin from Borden) in 55 g 2-methoxyethanol. 4.33 g of this dispersion was stirred into a solution made up of 3.7 g PD 140A resin, 0.35 g EC 2117 IR dye (available from FEW Wolfen GmbH), 30 mL methyl ethyl ketone and 30 mL 2-methoxyethanol and coated on a lithographic substrate to obtain 1.8 g/m² coating weight.
Second layer: 5 g of A-21 was dissolved on 100 mL toluene. The solution was stirred and then coated on top of the above mentioned first layer coated plate to give a coating weight of 1.0 g/m².

This plate was laser imaged on a Creo Trendsetter system as described in Example 1. Upon development with developer Goldstar from Kodak Polychrome Graphics, laser exposed areas of both first and second layers were removed without affecting the unexposed areas of either layer.

### EXAMPLE 9

A lithographic printing plate was prepared as follows:
First Layer: A polymeric solution was prepared by dissolving 1.25 g of 28-2930 copolymer, 1.25 g of Scriptset-550, 2.5 g of negative diazo N-5000 (condensation product of p-diazo diphenylamine bisulfate and formaldehyde isolated as the 2-hydroxy-4-methoxy benzophenone-5-sulfonate salt), and 0.9 g of ADS-830A IR dye into a solvent mixture containing 45 mL methyl ethyl ketone and 55 mL 2-methoxyethanol. The solution was spin coated on an electrolytically grained aluminum substrate to obtain a coating weight of 1.8 g/m².
Second layer: A solution containing 2.0 g of PMMA and 0.26 g of MP-1100 (polytetrafluoroethylene additive, available from DuPont Co.) in 100 g. toluene was coated on the above layer to obtain a coating weight of 0.6 g/m².

Two plates were imaged on the Creo Trendsetter thermal plate setter (wavelength 830 nm) at energy density between 140 and 240 mJ/cm². The plates were then developed with T-153 aqueous developer (from Kodak Polychrome Graphics) to produce printing plates having acceptable resolution.

One of the above developed plates was then flood exposed with UV radiation with a dose of 350 mJ/cm² using a SACK LCX3 5W source. Both the UV flood exposed and unexposed plates were then soaked for 2 min in developer T-153. The UV exposed plate exhibited higher resistance to developer and solvent.

### EXAMPLE 10

A lithographic printing plate was prepared as follows:
First Layer: 2.13 g of a carboxy-functional polyvinyl acetal (described in preparation example 11 of U.S. Patent 5,700,619 (T71 polymer), 2.13 g Nega 107 (a negative diazo resin derived from polycondensation of 3-methoxy-diphenylamine-4-diazonium sulfate and 4,4'-bis-methoxymethyldiphenyl ether, isolated as the mesitylene sulfonate salt, and available from Panchim) and 0.15 g EC 2117 IR 830 dye were dissolved in 50 mL of a solvent mixture of 2-methoxy-ethanol, methanol and methyl ethyl ketone (35: 25: 40). The solution was coated on an electrolytically grained, anodized and polyvinylphoshonic acid sealed substrate to obtain a coating weight of 1.4 g/m².
Second layer: A solution of 2 g nitrocellulose E950 (available from Wolff Walsrode) in 100 mL ethylacetate was coated on the above layer to give a coating weight of 1.1 g/m².

Two plates were laser imaged with a 810 nm laser diode mounted on a rotating drum to provide single lines and solid areas. The plates were then developed with aqueous alkaline developer 956 (from Kodak Polychrome Graphics) to obtain a good image with a clean background.

One of the plates was then flood exposed to UV radiation with a dose of 300 mJ/cm², using a SACK LCX3 5W radiation source. Both plates were soaked in diacetone alcohol for 15 minutes, resulting in a coating weight loss of 94% for the plate which was not flood exposed. The flood exposed plate had a weight loss of 46%, corresponding mainly to the loss of the nitrocellulose second layer. These results indicate that the photohardenable first layer was crosslinked during flood exposure.

### EXAMPLE 11

A lithographic printing plate was prepared as follows:
First Layer: A carbon dispersion AC 252 with 14.4% solid content was made by dispersing 20 g of T71 resin and 10 g carbon black (Spezialschwarz 250 from Degussa) in Dowanol PM. A coating solution was made up of 6.38 g of the dispersion, 0.41 g of T71 resin, 1.0 g of Nega 107 and 0.03 g of phosphoric acid in a solvent mixture of 2-methoxyethanol, methanol and methyl ethyl ketone (35: 25: 40). The solution was coated on an electrolytically grained, anodized and polyvinylphosphoric acid sealed substrate to obtain a coating weight of 1.0 g/m².
Second layer: A solution of 5 g PMMA in 100 mL toluene was coated on the above layer to give a coating weight of 0.5 g/m².

The plate was laser imaged with a 810 nm laser diode mounted on a rotating drum to obtain single lines and solid areas. The plate was then developed with aqueous alkaline developer 956 to obtain a good image with a clean background.

### EXAMPLE 12

A lithographic printing plate was prepared as follows:
First Layer: 5.1 g AK 128 (a polyvinylacetal containing dimethyl maleimido groups, described in DE 198 47 616.7 by Kodak Polychrome Graphics), 0.3 g Quantacure CPTX (thioxanthone derivative), 0.6 g EC 2117 IR 830 dye and 0.06 g 4-toluene sulfonic acid were dissolved in 80 mL of a solvent mixture of 2-ethoxyethanol, methanol and methyl ethyl ketone (35: 25: 40). The solution was coated on an electrolytically grained, anodized and polyvinylphosphonic acid sealed substrate to obtain a coating weight of 1.5 g/m².
Second layer: A solution of 5 g PMMA in 100 mL toluene was coated on the above layer to give a coating weight of 0.6 g/m².

Two plates were laser imaged with a 810 nm laser diode mounted on a rotating drum to provide single lines and solid areas. The plates were then developed with an aqueous alkaline developer 956 to obtain a good image with a clean background.

One of the plates was then flood exposed to UV radiation with a dose of 150 mJ/cm², using a SACK LCX3 5W radiation source. Both plates were soaked in diacetone alcohol for 15 minutes, resulting in a coating weight loss of 95% for the plate which was not flood exposed. The flood exposed plate had a weight loss of 37%, corresponding mainly to the loss of the PMMA second layer. These results indicate that the photohardenable first layer was crosslinked during flood exposure.

### EXAMPLE 13

A lithographic printing plate was prepared as follows:
First Layer: To the first layer solution of Example 12, 0.3 g of Nega 107 was added and the resulting solution coated on an electrolytically grained, anodized and polyvinylphosphonic acid sealed substrate to obtain a coating weight of 1.4 g/m².
Second layer: A solution of 5 g PMMA in 100 mL toluene was coated on the above layer to give a coating weight of 0.6 g/m².

Two plates were laser imaged with a 810 nm laser diode mounted on a rotating drum to provide single lines and solid areas. The plates were then developed with aqueous alkaline developer 956 to obtain a good image with a clean background.

One of the plates was then flood exposed to UV radiation with a dose of 150 mJ/cm², using a SACK LCX3 5W radiation source. Both plates were soaked in diacetone alcohol for 15 minutes, resulting in a coating weight loss of 93% for the plate which was not flood exposed. The flood exposed plate had a weight loss of 32%, corresponding mainly to the loss of the PMMA second layer. These results indicate that the photohardenable first layer was crosslinked during flood exposure.

## Claims

1. A positive-working thermal imaging element comprising:
A. a substrate; and
B. a thermally sensitive composite layer structure having an inner surface contiguous to the substrate and an outer surface, the composite layer structure comprising:
(a) a first layer having the inner surface, the first layer comprising a first polymeric material and a photothermal conversion material and wherein the first polymeric material is soluble or dispersible in an aqueous solution; and
(b) a second layer having the outer surface, the second layer comprising a second polymeric material, wherein the second layer is insoluble in the aqueous solution;
wherein the first layer, containing the photothermal conversion material, is applied first, and the second layer, not containing a photoconversion material, is subsequently applied; and wherein, upon imagewise heating of the composite layer structure, the composite layer structure is provided with heated portions and complementary unheated portions, wherein the heated portions have an increased rate of removal in the aqueous solution.

2. An imaging element according to claim 1, wherein the aqueous solution has a pH of 6 or greater.

3. An imaging element according to either of claims 1 and 2, wherein upon heating the composite layer structure, the first layer has an increased rate of dissolution or dispersibility in the aqueous solution.

4. An imaging element according to any one of the preceding claims, wherein upon heating the composite layer structure, the second layer has enhanced permeability to the aqueous solution.

5. An imaging element according to any one of the preceding claims, wherein the first polymeric material is insoluble in an organic solvent, and the second polymeric material is soluble in the organic solvent.

6. An imaging element according to any one of the preceding claims, wherein the first polymeric material is taken from the group consisting of carboxy functional acrylics, acrylics which contain phenol groups, acrylics which contain sulfonamido groups, cellulosic based polymers and copolymers, vinyl acetate/crotonate/vinyl neodecanoate copolymers, styrene maleic anhydride copolymers, polyvinyl acetals, phenolic resins, maleated wood rosin, and combinations thereof.

7. An imaging element according to claim 6, wherein the first polymeric material contains acid functionality derived from carboxylic acid groups, phenolic groups, sulfonamide groups or a combination thereof.

8. An imaging element according to any one of the preceding claims, wherein the first layer contains a photohardenable material activatable by actinic radiation.

9. An imaging element according to any one of the preceding claims, wherein the second polymeric material is selected from the group consisting of acrylic polymers and copolymers; polystyrene; styrene-acrylic copolymers; polyesters, polyamides; polyureas; polyurethanes; nitrocellulosics; epoxy resins; and combinations thereof.

10. A positive-working lithographic printing plate precursor which is the imaging element according to any one of the preceding claims wherein the substrate is a hydrophilic substrate; and the outer surface is an outer oleophilic surface.

11. A method for forming a planographic printing plate comprising the steps, in the order given:
I) providing the lithographic printing plate precursor according to claim 10;
II) imagewise exposing the composite layer structure to thermal energy to provide exposed portions and complementary unexposed portions in the composite layer structure, wherein the exposed portions are selectively removable by the aqueous solution; and
III) applying the aqueous solution to the outer oleophilic surface to remove the exposed portions to produce an imaged lithographic printing plate having uncovered hydrophilic areas of the hydrophilic substrate and complementary ink receptive areas of the outer oleophilic surface.

12. A method according to claim 11, wherein the first layer contains a photohardenable material activatable by actinic radiation wherein after step III, the imaged lithographic printing plate is uniformly exposed to ultraviolet radiation or to thermal energy.

## Patentansprüche

1. Positiv arbeitendes, thermisches Bildaufzeichnungselement, das umfasst:
A. ein Substrat; und
B. eine thermisch empfindliche Verbundschicht-Struktur mit einer inneren Oberfläche, die an das Substrat angrenzt, und einer äußeren Oberfläche,
wobei die Verbundschicht-Struktur umfasst:
a) eine erste Schicht mit der inneren Oberfläche, wobei die erste Schicht ein erstes polymeres Material und ein fotothermisches Konversionsmaterial umfasst und wobei das erste polymere Material in einer wässrigen Lösung löslich oder dispergierbar ist; und
b) eine zweite Schicht mit der äußeren Oberfläche, wobei die zweite Schicht ein zweites polymeres Material aufweist und in der wässrigen Lösung unlöslich ist;
wobei die erste Schicht, die das fotothermische Konversionsmaterial aufweist, zuerst aufgebracht wird und die zweite Schicht, die kein Fotokonversionsmaterial enthält, anschließend aufgebracht wird; und wobei bei einer bildweisen Erhitzung der Verbundschicht-Struktur die Verbundschicht-Struktur mit erhitzten Portionen und komplementären, unerhitzten Portionen versehen wird, wobei die erhitzten Portionen einen erhöhten Entfernungsgrad in der wässrigen Lösung aufweisen.

2. Bildaufzeichnungselement nach Anspruch 1, in dem die wässrige Lösung einen pH-Wert von 6 oder größer ausweist.

3. Bildaufzeichnungselement nach einem der Ansprüche 1 und 2, in dem bei Erhitzung der Verbundschicht-Struktur die erste Schicht einen erhöhten Grad an Löslichkeit oder Dispergierbarkeit in der wässrigen Lösung aufweist.

4. Bildaufzeichnungselement nach einem der vorstehenden Ansprüche, in dem bei Erhitzung der Verbundschicht-Struktur die zweite Schicht eine erhöhte Permeabilität gegenüber der wässrigen Lösung aufweist.

5. Bildaufzeichnungselement nach einem der vorstehenden Ansprüche, in dem das erste polymere Material in einem organischen Lösungsmittel unlöslich ist und das zweite polymere Material in dem organischen Lösungsmittel löslich ist.

6. Bildaufzeichnungselement nach einem der vorstehenden Ansprüche, in dem das erste polymere Material entnommen wird aus der Gruppe bestehend aus Acrylverbindungen mit funktionellen Carboxygruppen, Acrylverbindungen, die Phenolgruppen aufweisen, Acrylverbindungen, die Sulfonamidogruppen aufweisen, Polymeren und Copolymeren auf Cellulosebasis, Vinylacetat/Crotonat/Vinylneodecanoatcopolmyeren, Styrolmaleinsäureanhydridcopolymeren, Polyvinylacetalen, Phenolharzen, maleiertem Holzkolophonium und Kombinationen hiervon.

7. Bildaufzeichnungselement nach Anspruch 6, in dem das erste polymere Material eine Säurefunktionalität aufweist, die sich ableitet von Carboxylsäuregruppen, phenolischen Gruppe, Sulfonamidgruppen oder einer Kombination hiervon.

8. Bildaufzeichnungselement nach einem der vorstehenden Ansprüche, in dem die erste Schicht ein fotohärtbares Material enthält, das durch aktinische Strahlung aktivierbar ist.

9. Bildaufzeichnungselement nach einem der vorstehenden Ansprüche, in dem das zweite polymere Material ausgewählt wird aus der Gruppe bestehend aus Acrylpolymeren und -copolymeren; Polystyrol; Styrolacrylcopolymeren; Polyestern; Polyamiden; Polyharnstoffen; Polyurethanen; Nitrocellulosen; Epoxyharzen und Kombinationen hiervon.

10. Positiv arbeitender, lithografischer Druckplattenvorläufer, der das Bildaufzeichnungselement nach einem der vorstehenden Ansprüche darstellt, in dem das Substrat ein hydrophiles Substrat und die äußere Oberfläche eine äußere oleophile Oberfläche ist.

11. Verfahren zur Herstellung einer planografischen Druckplatte mit den folgenden Stufen in der angegebenen Reihenfolge:
I) Bereitstellung des lithografischen Druckplattenvorläufers gemäß Anspruch 10;
II) bildweise Exponierung der Verbundschicht-Struktur mit thermischer Energie zur Erzielung von exponierten Teilen und komplementären, unexponierten Teilen in der Verbundschicht-Struktur, wobei die exponierten Teile selektiv durch die wässrige Lösung entfernbar sind; und
III) Aufbringung der wässrigen Lösung auf die äußere oleophile Oberfläche unter Entfernung der exponierten Teile unter Erzeugung einer lithografischen Druckplatte mit einem aufgezeichneten Bild mit unbedeckten, hydrophilen Bereichen des hydrophilen Substrates und komplementären, Tinte aufnehmenden Bereichen der äußeren, oleophilen Oberfläche.

12. Verfahren nach Anspruch 11, bei dem die erste Schicht ein fotohärtbares Material aufweist, das durch aktinische Strahlung aktivierbar ist, wobei nach der Stufe III die lithografische Druckplatte mit dem aufgezeichneten Bild mit ultravioletter Strahlung oder thermischer Energie gleichförmig exponiert wird.

## Revendications

1. Elément formateur d'image thermique à effet positif comprenant :
A. un substrat ; et
B. une structure de couche composite thermosensible ayant une surface interne contiguë au substrat et une surface externe, la structure de la couche composite comprenant :
(a) une première couche ayant la surface interne, la première couche comprenant un premier matériau polymère et un matériau de conversion photothermique et où le premier matériau polymère est soluble ou dispersible dans une solution aqueuse ; et
(b) une seconde couche ayant la surface externe, la seconde couche comprenant un second matériau polymère, où la seconde couche est insoluble dans la solution aqueuse ;
où la première couche contenant le matériau de conversion photothermique est appliquée en premier et la seconde couche ne contenant pas de matériau de photoconversion est appliquée ultérieurement et où, après avoir chauffé la structure de la couche composite conformément à l'image, la structure de la couche composite comporte des parties chauffées et des parties complémentaires non chauffées, où les parties chauffées ont une vitesse d'élimination accrue dans la solution aqueuse.

2. Elément formateur d'image selon la revendication 1, dans lequel la solution aqueuse a un pH égal ou supérieur à 6.

3. Elément formateur d'image selon l'une ou l'autre des revendications 1 et 2, dans lequel, après avoir chauffé la structure de la couche composite, la première couche a une vitesse de dissolution ou de dispersibilité accrue dans la solution aqueuse.

4. Elément formateur d'image selon l'une quelconque des revendications précédentes, dans lequel, après avoir chauffé la structure de la couche composite, la seconde couche présente une meilleure perméabilité à la solution aqueuse.

5. Elément formateur d'image selon l'une quelconque des revendications précédentes, dans lequel le premier matériau polymère est insoluble dans un solvant organique et le second matériau polymère est soluble dans le solvant organique.

6. Elément formateur d'image selon l'une quelconque des revendications précédentes, dans lequel le premier matériau polymère est choisi parmi le groupe comprenant les acryliques ayant une fonction carboxy, les acryliques contenant des groupes phénol, les acryliques contenant des groupes sulfonamido, les polymères et les copolymères à base de cellulose, les copolymères d'acétate vinylique/de crotonate/de néodécanoate vinylique, les copolymères d'anhydride maléique et de styrène, les acétals polyvinyliques, les résines phénoliques, la résine de térébenthine maléée et leurs combinaisons.

7. Elément formateur d'image selon la revendication 6, dans lequel le premier matériau polymère contient une fonctionnalité acide dérivée des groupes acide carboxylique, des groupes phénoliques, des groupes sulfonamide ou d'une de leurs combinaisons.

8. Elément formateur d'image selon l'une quelconque des revendications précédentes, dans lequel la première couche contient un matériau photodurcissable pouvant être activé par rayonnement actinique.

9. Elément formateur d'image selon l'une quelconque des revendications précédentes, dans lequel le second matériau polymère est choisi parmi le groupe comprenant les polymères et les copolymères acryliques, le polystyrène, les copolymères acryliques et de styrène, les polyesters, les polyamides, les polyurées, les polyuréthanes, les nitrocelluloses, les résines époxy, et leurs combinaisons.

10. Précurseur de plaque d'impression lithographique à effet positif qui est l'élément formateur d'image selon l'une quelconque des revendications précédentes, dans lequel le substrat est un substrat hydrophile et la surface externe est une surface oléophile externe.

11. Procédé de formation d'une plaque d'impression planographique comprenant les étapes suivantes, dans l'ordre mentionné :
I) former le précurseur de la plaque d'impression lithographique selon la revendication 10 ;
II) exposer conformément à l'image la structure de la couche composite à l'énergie thermique pour former des parties exposées et des parties non exposées complémentaires dans la structure de la couche composite, où les parties exposées sont sélectivement éliminables par la solution aqueuse ; et
III) appliquer la solution aqueuse sur la surface oléophile externe pour éliminer les parties exposées afin de produire une plaque d'impression lithographique imagée comportant des zones hydrophiles non revêtues du substrat hydrophile et des zones complémentaires réceptrices d'encre de la surface oléophile externe.

12. Procédé selon la revendication 11, dans lequel la première couche contient un matériau photodurcissable pouvant être activé par rayonnement actinique, dans lequel après l'étape III, la plaque d'impression lithographique imagée est uniformément exposée au rayonnement ultraviolet ou à l'énergie thermique.
